# EUROPEAN PATENT SPECIFICATION

(11) **EP 0 042 702 B1**
(45) Date of publication and mention of the grant of the patent: **26.09.1984**
(21) Application number: 81302614.3
(22) Date of filing: 12.06.1981
(51) Int. Cl.: C22B 13/00, C22B 11/00

(54) **Process for the recovery of lead and silver from minerals and process residues**
Verfahren zur Rückgewinnung von Blei und Silber aus Erzen und Rückständen
Procédé pour la récupération de plomb et d'argent à partir de résidus

(30) Priority: 16.06.1980 CA 354083
(43) Date of publication of application: 30.12.1981
(73) Proprietor: Provincial Holdings Ltd., Fredericton New Brunswick E3B 5H1 (CA)
(72) Inventor: Salter, Robert Steven, Fredericton, New Brunswick (CA); Boorman, Roy Slater, Fredericton New Brunswick (CA); Gilders, Ross David, Fredericton, New Brunswick (CA)
(74) Representative: Dew, Melvyn John

## Description

This invention relates to the extraction of metal compounds from metal bearing materials and more particularly to the extraction and recovery of lead values in a calcium plumbate and/or oxide product from minerals or lead bearing materials. Silver which may be present in association with the lead may be recovered as native silver, silver chloride, sulfide or sulphate, or a silver complex with other metals, or in some other form from which it can be recovered by conventional techniques.

The recovery of a high grade lead product suitable for treatment for metal recovery from lead bearing minerals has usually been accomplished by flotation concentration of coarse grained lead sulphide deposits into a concentrate containing greater than 50% lead and pyrometallurgical reduction of this concentrate in a blast furnace. The reserves of these coarse grained lead sulphide deposits are rapidly being depleted. The major new reserves of lead are being found in fine grained massive sulphide deposits containing sulphides of zinc, lead, copper, silver, and iron. Recoveries into high grade lead concentrates are typically low from these deposits, necessitating significant reduction in grade to maintain economic recoveries. It will be necessary for some of these deposits to resort to the production of bulk zinc, lead, copper concentrates to insure high recoveries. Several new processes are available for treating these low grade and bulk type concentrates including ferric chloride leach processes, copper chloride leach processes, sulphuric acid-oxygen pressure leach processes and the sulphation roast process. The lead and silver in the latter two processes report in a low grade lead sulphate-hematite leach residue. In the ferric and cupric chloride leach processes, leach filtrates are produced which contain lead and silver as chlorides in a concentrated brine solution. The present process has application for lead and silver recovery from the leach residues and brine solutions generated in all of these processes.

Substantial reserves of lead and silver also exist in leach residues from electrolytic zinc plants. These residues typically assay 15-40% lead as lead sulphate and for the most part are considered as unsuitable as feed for a conventional lead smelter except in small amounts. Another source of low grade materials is slag from lead smelters. Lead is presently recovered from these slags by energy intensive fuming processes. The present process can be employed directly to recover lead and silver from zinc plant residues and after either sulphuric acid leaching or sulphation roasting to recover lead and silver from slags.

It is known that lead sulphate and associated silver may be solubilized by means of concentrated brines as proposed in Canadian Patent 19,918, (1883); Canadian Patent 228,518, (1919); and U.S. Bureau of Mines Bulletin 157, (1918). Whilst these methods solve the problem of separating the lead and silver from the residues there has been some economic difficulty in the subsequent recovery of the lead and silver from the solution in a usable form.

West German Patent 2,500,453, (1976) describes a method of leaching lead sulphate containing material in sodium chloride solution and after residue separation, precipitating the Pb from solution with milk of lime. The lead precipitates contain greater than 10% chloride and 11% sulphate and are not acceptable to conventional lead smelters except in small amount and at depressed prices due to the deleterious effects of chlorides on acid plant catalysts, baghouses, and refractories.

Canadian Patent 228,518, (1919); United States Patent 4,063,933, (1977); and processes currently being developed by the U.S. Bureau of Mines, Minemet Recherche, (France), and Cominco Limited (Canada), advocate lead recovery by the precipitation of lead chloride crystals from solution by evaporation and/or cooling. The subsequent recovery of lead metal to be accomplished by electrolysis. Capital and operating costs are projected to be much higher for these processes than for conventional smelting.

Australian Patent 28,957, (1971) describes a method of precipitating lead chloride from brine solution by cooling followed by reacting said lead chloride with water and calcium sulphate to produce a lead sulphate precipitate and calcium chloride solution. Although low chloride levels in the lead sulphate were obtainable with rigorous washing, the product is again suitable to lead smelters in limited quantities and must be treated on a sinter machine to remove sulphur before the blast. Capital and operating costs are projected to be high for the process since the brine solution must be heated for high lead solubility and then cooled for lead chloride precipitation.

Canadian Patent 228,518, (1919) describes a method of lead recovery from concentrated brine solution by direct precipitation as sulphide or sulphate. These precipitates are difficult to wash and contain significant amounts of entrapped chlorides. Again conventional lead smelters will accept only small quantities.

Canadian Patent 19,918 describes a method of precipitating lead and silver from brine solution by cementation on metallic zinc. Recently other researchers have rediscovered the cementation technique and advocate either zinc or iron as cementation media. High grade metallic lead and silver cementates are produced in these processes which are acceptable to lead smelters at premium prices at high tonnage. Considerable economic penalties are incurred to produce good quality cementates, however, since the cementation reagents are expensive and the zinc or iron in the lean brine resulting from cementation must be recovered in a form acceptable for sale or reuse. This can be accomplished only at considerable cost.

French Patent 2,297,253 describes a process for recovery of lead values which comprises (a) preparing a solution of lead chloride by treatment of a lead sulphate-containing material with a chloride- containing solution; (b) removing insoluble material from the solution thus obtained; (c) precipitating lead oxychloride from the solution by the addition of lime; (d) separating the precipitate thus formed; and (e) fusing the precipitate with lime, carbon and iron to recover the lead.

It is an objective of this invention to provide a process for the extraction and recovery of lead and silver into a product which will be acceptable to conventional lead smelters in large tonnages and at a premium price.

Further objectives are for the process to consume minimum energy and the reagents used to be recovered and either reused with high efficiency or credited in the sale of the lead product.

According to one aspect of this invention there is provided a process for gaining lead and silver values comprising the steps of (a) preparing a solution of lead chloride and silver compounds by dissolving lead sulphate and silver compounds contained in an ore or process residue in an acidic concentrated chloride brine; (b) separating the solution so formed from insoluble gangue or other residue; and (c) forming a precipitate of lead oxychloride and silver compounds by adding lime to said solution and separating said precipitate from the residual lean brine solution, characterised by the further steps of (1) reacting the said oxychloride precipitate with oxygen and lime in a reactor at an elevated temperature to produce a calcine containing most of the lead as calcium plumbates and/or lead oxides and most of the silver as silver or silver compounds; (2) washing said calcine in water and/or dilute chloride brine to dissolve soluble chlorides; and (3) separating the resulting residue containing calcium plumbates and/or lead oxides, as well as silver and silver compounds, from the resulting chloride brine.

Step (a) is preferably performed at a temperature in the range 30°C to the boiling point of the chloride brine, at a pH between 1.5 and 4.5, and a retention time of 0.5-2.5 hours. The chloride brine advantageously comprises a solution of one or more inorganic chlorides in water, which at room temperature is saturated or nearly saturated. In step (c), the mole ratio of lime to lead is advantageously from 0.75 to 5.5, and preferably 1.5; the retention time is advantageously 0.5-2.5 hours and the temperature in the range 30°C to the boiling point of the chloride brine.

In one embodiment, part of the silver is recovered from the lead sulphate containing material by flotation prior to step (a). Silver may be recovered between steps (b) and (c) by cementation on one of metallic zinc, iron, or lead. Silver and lead, or lead alone, may be recovered in the residue from step (3).

In step (1), the lime reacted with the oxychloride precipitate is advantageously such as to increase the total lime additions in step (c) and step (1) to between 1.75 and 5.5, preferably 3.0, mole ratio to lead. The lime in step (a) may in fact be constituted by excess lime present in the precipitate from step (c); fresh lime may be added to supplement the excess lime in the precipitate from step (c). The mole ratio of oxygen to lead in step (1) is preferably in excess of 0.5.

According to a second aspect of the invention there is provided a process for gaining lead values, comprising forming a precipitate of lead oxychloride by adding lime to a chloride brine solution containing lead chloride, and separating said lead oxychloride from the residual lean brine solution, characterised by the steps of (1) reacting the said precipitate with oxygen and lime in a reactor at an elevated temperature to produce a calcine containing most of the lead as calcium plumbates and/or lead oxides; (2) washing said calcine in water and/or dilute chloride brine to dissolve soluble chlorides; and (3) separating the resulting residue containing calcium plumbates and/or lead oxides from the resulting chloride brine.

The residue obtained in step (3) is preferably washed with fresh water to remove residual chlorides. The chloride brines resulting from the various process steps can be recycled for reuse in the process.

The chloride brine advantageously comprises calcium chloride, preferably with a mole ratio of calcium chloride to lead sulphate greater than 4. The chloride brine may also include one or both of sodium and magnesium chloride.

Step (1) is preferably performed at a temperature above 325°C for longer than 0.5 hours, more preferably at 400°C for 1.0 hours. The oxygen is conveniently in the form of air.

The invention will now be explained in greater detail with reference to the accompanying drawings, in which:
Figure 1 is a schematic flow sheet showing certain aspects of the present invention;
Figure 2 is a graph showing the relationship between calcium chloride addition and sulphate in solution;
Figure 3 is a schematic flow sheet showing a lead-silver receovery plant employing certain aspects of this invention.

The advantages of producing a calcium plumbate product are as follows:
i) calcium plumbate is not water or cold brine soluble and will not react with chloride brines under neutral or basic conditions to reform lead oxychlorides.
ii) entrained chlorides in the plumbate calcine can be easily removed and reduced to very low levels by washing with water or unsaturated brine solution.
iii) plumbate repulp solutions filter rapidly, leaving a dry residue.
iv) plumbate products can be briquetted and fed directly into a lead smelter blast furnace without prior sintering, increasing smelter throughput for smelters in which the capacity is limited by the sinter machine.
v) as reported by Denev, D.G. et al in Dokl. Bolg. Akad. Nauk, Vol. 26, 11, 1973, page 1485 calcium orthoplumbate is an oxidant for lead sulphide at high temperature resulting in the products PbO, CaO and S0₂ and hence would make a good dilutant for galena concentrate on a sinter machine.
vi) CaO is a product of the reduction of calcium plumbate and is also required as a slagging agent in lead blast furnaces, usually at high tonnages. Accordingly, since the use of some calcium plumbate as feed to a lead smelter would reduce the requirement for lime, some credit should be given for the lime in the plumbate product.
vii) the production of a calcium plumbate product allows for the use of lime for the precipitation of the lead from the brine leach solution and also as a reactant in the high temperature conversion of oxychloride to plumbate. Lime is a relatively inexpensive, easy to handle, environmentally acceptable, and readily available commodity.
viii) the use of lime results in the formation of calcium chloride after the conversion of the metal chlorides (lead, zinc, copper, iron) to oxides. This calcium chloride is recycled in the brine to the lead sulphate leach and results in the precipitation of most of the sulphate as calcium sulphate into the leach residue. Accordingly the plumbate product is low in sulphate. Also, the low soluble sulphate in the leach enhances the solubility of lead and silver allowing for leach operation at lower temperatures, resulting in a lower energy consumption and less maintenance due to decreased corrosion. The effect of calcium chloride on sulphate solubility in sodium chloride brine solution is shown in Figure 2. The solubility of lead as lead sulphate in 269 gpl NaCI brine increases from about 13 gpl at 35°C to about 18 gpl (grams per liter) at 35°C when CaCI₂ is added to yield a brine containing 34 gpl CaCt:,. Lead solubility is directly proportional to the brine saturation and the sulphate concentration in the brine.

Since calcium chloride is a more expensive commodity than sodium chloride and since there appears to be a lower limit to the soluble sulphate in the brine leach solution attainable with calcium chloride and since sodium chloride is easier to remove from leach residue by washing, it seems to be preferable but not necessary to use a concentrated sodium chloride brine as the base solution using the lime additions in steps (3) and (5) as the source of calcium chloride for sulphate removal. Small amounts of fresh NaCI and CaCI₂ will be required to make up for losses in the leach residue and product.

Lead and silver extractions into brine can be accelerated by increasing the acidity by addition of an acid such as hydrochloric or sulfuric acid which will ensure at least mildly acidic conditions. The optimum pH in the brine leach for high lead and silver extraction, efficient residue washing, and low lime consumption appears to be about 1.5.

Extractions of lead from lead sulphate material into brine are very high and may approach 99% with the proper choice of retention time, temperature, brine composition, and residue washing techniques as long as the solubility limit of the lead is not approached. Lead extractions fall from 99% at 75% of lead chloride saturation to 96% at 86% of saturation to 91 % at 94% of saturation for brine leaching in 269 gpl NaCl - 33 gpl CaCI₂ - pH 1.5 brine at 35°C and 1.5 hours leaching time. The saturation limit of lead as lead chloride in this brine is 18.3 gpl.

Silver extraction by brine is very dependent on the nature and prior history of the lead sulphate containing material. Some materials, usually those which have been very recently produced in a roaster or leach process exhibit silver extractions greater than 80%. Other materials, usually stockpiled, exhibit lower silver extractions of about 50%. Silver recoveries can be increased from these materials by flotation recovery of a silver concentrate and using the present process on the flotation tailings which contain most of the lead and all the remaining silver. The silver flotation concentrate and the plumbate product can then be combined for sale to conventional lead smelters. Flotation processes such as described by Moriyama, E. and Yamamoto, Y. in AIME World Symposium of Mining and Metallurgy of Lead and Zinc, Vol. II, 1970, page 215 have been shown to yield silver concentrates with high silver assays and recoveries from lead sulphate containing materials.

Another option in the present process is the production of separate silver and lead products. Silver can be removed from the brine leach solution by cementation on a suitable metallic medium such as zinc, iron, or lead. With proper stoichiometric conditions, retention time, and pH nearly all the silver can be recovered in a high grade metallic product containing some little lead and copper as contaminants. Lead along with the solubilized cementation agent would then be recovered in the plumbate product as in steps (3)-(9).

When lead is precipitated from brine solution by the addition of a base as in step (3) of the process, the lead compounds formed will depend on the pH or the mole ratio of base to lead chloride and the total chloride concentration. Table 1 shows the effect of these variables on the nature of the lead precipitate when lead is precipitated from a brine solution containing 15 gpi lead as lead chloride at 45°C and a retention time of 1.5 hours. Shorter retention times can be employed but chloride levels in the precipitate will increase unless the temperature is increased above 45°C. Silver is coprecipitated with lead. Most of the brine soluble impurities which are present in the lead sulphate containing starting material such as zinc, copper, iron, bismuth, and arsenic also coprecipitate with lead. The best process economics are obtained with lime as the precipitation agent at an addition rate between 1.0 and 5.5 mole ratio of lime to lead chloride. The excess lime also acts as flocculating agent for oxychloride precipitate,

resulting in improved solid/liquid separation.

Although it is desirable to produce a precipitate containing as little chloride as possible, very low chloride-oxychlorides cannot be precipitated from concentrated brine unless uneconomic quantities of sodium hydroxide are used. Since they are very soluble, all excess sodium hydroxide and/or sodium carbonate must be neutralized with hydrochloric acid before the lean brine resulting from precipitate separation can be recycled to the brine leach step (1). The use of sodium hydroxide precipitating agent also results in excessive reagent calcium chloride makeup requirements.

Ermilov, V.V. and Aitenov, S.A. in Trudy Institut Metallurgi Obogashcheniia, Vol. 30, 1969, page 47 proposed a method for producing a lead (iv) oxide precipitate from concentrated brine by adding equal molar quantities of calcium oxide and calcium hypochlorite to lead chloride. Although the reaction is irreversible and regenerates calcium chloride into solution, and the product can easily be washed to less than 0.5% chloride, the economics are unfavourable due to the value of hypochlorite in comparison to lead metal and lime.

If the lime addition in the precipitation step (3) was less than 2.5 mole ratio to lead, then after separation of the lead oxychloride precipitate from the lean brine solution, the precipitate is repulped with water or any reasonably unsaturated brine solution produced in the process. Lime is added to the pulp to bring the mole ratio of the total lime addition in the process to between 2.5 and 5.5. After solid/liquid separation the pulp is subjected to thermal treatment. Alternatively the lead oxychloride precipitate may be blended with lime to increase the total mole ratio to between 2.5 and 5.5, without repulping and the blend subjected to thermal treatment.

If the lime addition in step (3) was greater than 2.5 mole ratio to lead, then repulping and/or further lime addition is not necessary before thermal treatment.

The lead oxychloride-lime blend is heated in a reactor in the presence of oxygen or air. The reactor can be a rotary kiln, furnace, roaster, autoclave or any device commonly used for thermal treatment. The retention time in the reactor depends upon the desired degree of conversion of oxychloride to plumbate and oxide, the temperature in the reactor, the lime to lead mole ratio, and the oxygen partial pressure. The effects of these variables on the nature of the calcine product are shown in Table 2. At reaction temperatures above 500°C sintering of the product appears and volatilization of lead chloride begins. Preferred conditions appear to be a total process lime addition to lead mole ratio of about 3, a reaction temperature of about 400°C, a retention time of about 1 hour, and an excess of oxygen for lead oxidation. Pressure above atmospheric is not required for the reaction to be complete within 2

hours. Sufficient air or oxygen can be supplied for the reaction by convection, free or forced, or by pressurizing the reactor.

It is surprising that calcium orthoplumbate (Ca₂PbO₄ is formed at high yields with such low temperatures and short retention times. Calcium orthoplumbate in a pure form (>90%) is a valuable commodity and is used in the manufacture of primers for steel and galvanized steel, of pigments and of binders for paints. It also has use in the plastics and resin industries. The common commercial production method is the reaction of PbO with lime and air or oxygen at temperatures above 700°C. The reaction kinetics are reportedly slow below this temperature and the reaction will not go below 500°C. It has been reported by Denev, D.G. et al in Dokl. Bolg. Akad. Nauk, Vol. 26, 11, 1973, page 1485, however, that additions of small quantities of NaCI to the reaction mixture speed the kinetics. The present invention differs from the customary practice in that the reagent for calcination is lead oxychloride and not lead oxide. Also, the oxychloride is contaminated with significant quantities of NaCl and CaCI2. Accordingly, the kinetics and energetics of plumbate formation have been altered significantly from commercial experience.

Figure 3 is a schematic plant layout for a particular embodiment of the invention relating to example 1.

The following examples illustrate the practice of our invention but should not be construed as limiting.

### Examples 1 to 8 inclusive

Samples of hot sulphuric acid leach residues obtained from the sulphation roasting and leaching of bulk zinc-lead-copper-silver sulphide concentrates assaying 30-32% Zn, 3.5-10% Pb, 0.7% Cu, 4.4-8.8 oz/ST (troy ounce per short ton) silver, and 14-23% iron were processed accordingly to the invention. A sample (example 10) of a hot acid leach residue from a dead roast zinc plant was also processed. The residues assayed as in Table 3.

The residues were leached in brines of composition given in Table 4. Residue was added at a ratio of 15 gm of contained lead per litre of brine. The leaches were conducted at 35-40°C for 1.5 hours. Leach residues were allowed to settle and the thickened residues filtered and washed with fresh brine. Extractions of lead and silver are given in Table 5. All of the zinc, iron and copper as sulphates in the hot sulphuric acid leach residues leached along with the lead and silver. Copper and bismuth assays in the brine were 40 and 45 mgpl respectively.

One pregnant brine solution (example #6) was treated with zinc dust at an addition rate of 0.5 gpl producing a cementate containing 99% of the silver, 95% of the copper and 80% of the bismuth in the pregnant brine.

The remaining pregnant brines and the solution resulting from the zinc dust cementation test were then treated with lime at 1.5 mole ratio to lead in the brine solution. The temperature and retention time were 45°C and 1.5 hours respectively.

Precipitates were allowed to settle and the thickened precipitates filtered.

The precipitates in all tests were then blended with lime, as required, to bring the total mole ratio of lime added to the process to lead in the precipitate to 1.75-5.5. The blends were

treated in an oven with a slow purge of fresh air for 1.0 hours at 400°C. The calcines were repulped to 50% pulp density for 15 minutes in fresh water and filtered and displacement washed with a volume of water equal to the calcine repulp water. The assays (dry basis) of the resulting plumbate products are given in Table 6.

### Example 11

A sample of the hot sulfuric acid leach residue used in example 5 was repulped in water at 10% pulp density, American Cyanamid flotation reagents Aero 404 (trade mark) promoter and Aerofroth 77A (trade mark) (frother) were added at 600 g and 60 g per metric ton of residue respectively. After 5 minutes conditioning time, flotation was initiated and a stable froth was maintained for about 7.5 minutes. The concentrate obtained assayed 18% Pb, 24% Fe, 1.8% Zn, and 635 oz/ST silver. Silver recovery from the head material was 70%.

The tailings from the flotation were treated in the process exactly similar to example 4. Silver recovery from the tailings was 35%, resulting in an overall silver recovery of 81%.

As will be apparent to those skilled in this art, the process of this invention may be applied to the recovery of metals from a variety of metallurgical products such as ores and concentrates, smelter dusts, metal drosses, middling concentrates from flotation processing, slags and process residues, and other like sources of iead and silver.

## Claims

1. A process for gaining lead and silver values comprising the steps of (a) preparing a solution of lead chloride and silver compounds by dissolving lead sulphate and silver compounds contained in an ore or process residue in an acidic concentrated chloride brine; (b) separating the solution so formed from insoluble gangue or other residue; and (c) forming a precipitate of lead oxychloride and silver compounds by adding lime to said solution and separating said precipitate from the residual lean brine solution, characterised by the further steps of (1) reacting the said oxychloride precipitate with oxygen and lime in a reactor at an elevated temperature to produce a calcine containing most of the lead as calcium plumbates and/or lead oxides and most of the silver as silver or silver compounds; (2) washing said calcine in water and/or dilute chloride brine to dissolve soluble chlorides; and (3) separating the resulting residue containing calcium plumbates and/or lead oxides, as well as silver and silver compounds, from the resulting chloride brine.

2. A process according to claim 1 characterised in that step (a) is performed at a temperature in the range 30°C to the boiling point of the chloride brine, at a pH between 1.5 and 4.5, and a retention time of 0.5-2.5 hours.

3. A process according to claim 1 or 2, characterised in that step (c) is performed by adding lime at a mole ratio of between 0.75 and 5.5, preferably 1.5, to dissolved lead.

4. A process according to claim 1, 2 or 3 characterised in that step (c) is performed for a retention time between 0.5 and 2.5 hours and the temperature is in the range 30°C to the boiling point of the chloride brine.

5. A process according to any one of the preceding claims characterised in that step (1) is performed by adding lime to the said oxychloride precipitate to increase the total of the lime additions in step (c) and step (1) to between 1.75 and 5.5, preferably 3.0, mole ratio to lead.

6. A process according to claim 1, 2, 3, 4 or 5, characterised in that lead and silver are recovered in the residue from step (3).

7. A process according to claim 1, 2, 3, 4 or 5, characterised in that lead is recovered in the residue from step (3).

8. A process according to any one of the preceding claims, characterised in that silver is recovered by cementation on one of metallic zinc, iron, or lead between step (b) and step (c).

9. A process according to any one of the preceding claims characterised in that a portion of the silver is recovered from the lead sulphate containing material by flotation prior to step (a).

10. A process according to any one of the preceding claims characterised in that step (1) is performed with a mole ratio of oxygen to lead in excess of 0.5.

11. A process according to any one of the preceding claims characterised in that the concentrated chloride brine comprises a saturated or nearly saturated solution at room temperature of one or more inorganic chlorides in water.

12. A process according to any preceding claim characterised in that the lime in step (1) is excess lime present in the precipitate from step (c).

13. A process according to claim 12 characterised in that in step (1) fresh lime is added to supplement the excess lime present in the precipitate from step (c).

14. A process for gaining lead values, comprising forming a precipitate of lead oxychloride by adding lime to a chloride brine solution containing lead chloride, and separating said lead oxychloride from the residual lean brine solution, characterised by the steps of (1) reacting the said precipitate with oxygen and lime in a reactor at an elevated temperature to produce a calcine containing most of the lead as calcium plumbates and/or lead oxides; (2) washing said calcine in water and/or dilute chloride brine to dissolve soluble chlorides; and (3) separating the resulting residue containing calcium plumbates and/or lead oxides from the resulting chloride brine.

15. A process according to claim 14, characterised in that the chloride brine solution is any chloride brine solution containing lead chloride.

16. A process according to any one of the preceding claims, wherein the residue obtained in step (3) is washed with fresh water to remove residual chlorides.

17. A process according to any one of the preceding claims characterised in that one component of the chloride brine is calcium chloride.

18. A process according to claim 17, characterised in that the chloride brine comprises an aqueous solution of calcium chloride and one or both of sodium and magnesium chloride.

19. A process according to any one of the preceding claims characterised in that the chloride brine includes calcium chloride, and in that the mole ratio of calcium chloride to lead sulphate is greater than 4.

20. A process according to any one of the preceding claims characterised in that step (1) is performed at a temperature above 325°C for longer than 0.5 hours, preferably at 400°C for 1.0 hour.

21. A process according to any one of the preceding claims characterised in that the oxygen is in the form of air.

22. A process according to any one of the preceding claims characterised in that the chloride brines resulting from the steps are recycled for re-use in the process.

## Revendications

1. Procédé pour la valorisation des résidus industriels de plomb et d'argent comprenant des opérations de: (a) la préparation d'une solution de composés d'argent et de chlorure de plomb par dissolution dans une saumure concentrée acide de chlorures des composés d'argent et de sulfate de plomb contenus dans un minerai ou dans un résidu de procédé; (b) la séparation de la solution ainsi formée de la gangue insoluble ou d'un autre résidu; (c) la formation d'un précipité de composés d'argent et d'oxychlorure de plomb par addition de chaux à cette solution et la séparation du précipité de la solution de saumure résiduelle pauvre, caractérisé par les opérations supplémentaires: (1) la reaction du précipité d'oxychlorure avec de l'oxygène et de la chaux dans un réacteur à une température élevée pour obtenir un calcin contenant la plupart du plomb sous forme de plombates de calcium et/ou d'oxydes de plomb et la plupart de l'argent sous forme d'argent ou de composés d'argent; (2) le lavage de ce calcin dans de l'eau et/ou de la saumure diluée de chlorure pour dissoudre les chlorures solubles; (3) la séparation du résidu résultant contenant des plombates de calcium et/ou des oxydes de plomb ainsi que l'argent et des composés d'argent, à partir de la saumure de chlorures résultante.

2. Procédé selon la revendication 1 caractérisé en ce que l'opération (a) est exécutée à une température comprise dans la gamme de 30°C au point d'ébullition de la saumure de chlorure, à un pH compris entre 1,5 et 4,5, avec une durée de séjour de 0,5 à 2,5 heures.

3. Procédé selon l'une quelconque des revendications 1,2 caractérisé en ce que l'opération (c) est exécutée par addition de chaux à un rapport molaire compris entre 0,75 et 5,5, de préférence 1,5, par rapport au plomb dissous.

4. Procédé selon l'une quelconque des revendications 1 à 3 caractérisé en ce que l'opération (c) est exécutée pendant une durée de séjour comprise entre 0,5 et 2,5 heures et la température est comprise dans la gamme de 30°C au point d'ébullition de la saumure de chlorure.

5. Procédé selon l'une quelconque des revendications 1 à 4 caractérisé en ce que l'opération (1) est exécutée par addition de chaux audit précipité d'oxychlorure pour augmenter le total des additions de chaux pendant l'opération (c) et l'opération (1) jusqu'à un rapport molaire par rapport au plomb compris entre 1,75 et 5,5, de préférence 3.

6. Procédé selon l'une quelconque des revendications 1 à 5 caractérisé en ce que le plomb et l'argent sont récupérés dans le résidu à partir de l'opération (3).

7. Procédé selon l'une quelconque des revendications 1 à 5 caractérisé en ce que le plomb est récupéré dans le residu a partir de l'opération (3).

8. Procédé selon l'une quelconque des revendications 1 à 7 caractérisé en ce que l'argent est récupéré par cémentation sur l'un des métaux zinc, fer ou plomb entre l'opération (b) et l'opération (c).

9. Procédé selon l'une quelconque des revendications 1 à 8 caractérisé en ce qu'une partie de l'argent est récupérée de la matière contenant du sulfate de plomb par flottation avant l'opération (a).

10. Procédé selon l'une quelconque des revendications 1 à 9 caractérisé en ce que l'opération (1) est exécutée avec un rapport molaire de l'oxygène par rapport au plomb en excès de 0,5.

11. Procédé selon l'une quelconque des revendications 1 à 10 caractérisé en ce que la saumure concentrée de chlorures comprend une solution saturée ou presque saturée à la température de l'environnement d'un ou de plusieurs chlorures inorganiques dans de l'eau.

12. Procédé selon l'une quelconque des revendications 1 à 11 caractérisé en ce que la chaux de l'opération (1) est de la chaux en excès présente dans le précipité provenant de l'opération (c).

13. Procédé selon la revendication 12 caractérisé en ce que dans l'opération (1) on ajoute de la chaux fraîche en supplément à la chaux en excès présente dans le précipité provenant de l'opération (c).

14. Procédé pour valoriser des résidus de plomb comprenant la formation d'un précipité d'oxychlorure de plomb par addition de chaux à une solution de saumure de chlorure contenant du chlorure de plomb, et la séparation de cet oxychlorure de plomb de la solution de saumure résiduelle pauvre, caractérisé par les opérations de: (1) la réaction de ce précipité avec de l'oxygène et de la chaux dans un reacteur à une température élevée pour donner un calcin contenant la plupart du plomb sous forme de plombates de calcium et/ou d'oxydes de plomb; (2) le lavage de ce calcin dans de l'eau et/ou de la saumure de chlorure diluée pour mettre en solution les chlorures solubles; (3) la séparation de la saumure de chlorure résultante du résidu obtenu contenant des plombates de calcium et/ou des oxydes de plomb.

15. Procédé selon la revendication 14 caractérisé en ce que la solution de saumure de chlorure est une solution contenant du chlorure de plomb.

16. Procédé selon l'une quelconque des revendications 1 à 15 caractérisé en ce que le résidu obtenu à l'opération (3) est lavé avec de l'eau fraîche pour l'élimination des chlorures résiduels.

17. Procédé selon l'une quelconque des revendications 1 à 16 caractérisé en ce que l'un des composants de la saumure de chlorures est du chlorure de calcium.

18. Procédé selon la revendication 17 caractérisé en ce que la saumure de chlorures comprend une solution aqueuse de chlorure de calcium et l'un ou les deux des chlorures de sodium et de magnésium.

19. Procédé selon l'une quelconque des revendications 1 à 18 caractérisé en ce que la saumure de chlorures comprend du chlorure de calcium et en ce que le rapport molaire du chlorure de calcium au sulfate de plomb est supérieur à 4.

20. Procédé selon l'une quelconque des revendications 1 à 19 caractérisé en ce que l'opération (1) est exécutée à une température supérieure à 325°C pendant plus de 0,5 heure, de préférence à 400°C pendant 1 heure.

21. Procédé selon l'une quelconque des revendications 1 à 20 caractérisé en ce que l'oxygène est sous forme d'air.

22. Procédé selon l'une quelconque des revendications 1 à 21 caractérisé en ce que les saumures de chlorures résultantes des opérations sont recyclées pour réutilisation dans le procédé.

## Patentansprüche

1. Verfahren zum Erschließen von Blei- und Silber- Beständen (Vorräten, values) umfassend die Stufen
(a) Herstellen einer Lösung von Bleichlorid und Silberverbindungen durch Auflösen von in einem Erz oder Prozeßrückständen enthaltenem Bleisulfat und Silberverbindungen in einer sauren konzentrierten Chloridlösung,
(b) Abtrennen der so gebild eten Lösung von unlöslichem Ganggestein oder andren Rückständen und
(c) Ausfällen von Bleioxichlorid und Silberverbindungen durch Zugabe von Kalk und Abtrennen des Niederschlags von der verbleibenden mageren Salzlösung, gekennzeichnet durch die weiteren Stufen

(1) Behandeln des besagten Oxichloridniederschlags mit Sauerstoff und Kalk in einem Reaktor bei erhöhter Temperatur zur Herstellung eines Kalzinats (calcine), welches das meiste Blei als Calciumplumbat und/oder Bleioxid sowie das meiste Silber in Form von Silber oder Silberverbindungen enthält,

(2) Waschen des Kalzinats mit Wasser und/oder verdünnter Chloridlösung zum Herauslösen der löslichen Chloride und

(3) Abtrennen des erhaltenen Rückstandes mit Calciumplumbat und/oder Bleioxid sowie Silber und Silberverbindungen von der Salzlösung.

2. Verfahren nach Patentanspruch 1, dadurch gekennzeichnet, daß in der Stufe (a) die Temperatur zwischen 30°C und dem Siedepunkt der Chloridlösung liegt, der pH-Wert zwischen 1,5 und 4,5 beträgt und die Behandlungsdauer 0.5-2,5 Stunden ist.

3. Verfahren nach Patentanspruch 1 oder 2, dadurch gekennzeichnet, daß in der Stufe (c) die Zugabe vom Kalk in einem Molverhältnis zwischen 0,75 und 5,5, vorzugsweise 1,5, zum gelösten Blei erfolgt.

4. Verfahren nach Patentanspruch 1, 2 oder 3, dadurch gekennzeichnet, daß in der Stufe (c) die Behandlungsdauer zwischen 0,5 und 2,5 Stunden liegt und die Temperatur von 30°C bis zum Siedepunkt der Chloridlösung beträgt.

5. Verfahren nach einem der vorherigen Ansprüche, dadurch gekennzeichnet, daß in der Stufe (1) der Zusatz vom Kalk zu dem Oxichloridniederschlag in einer solchen Menge erfolgt, daß die Gesamtzugabe von Kalk in den Stufen (c) und (1) im Molverhältnis zu Blei zwischen 1,75 und 5,5, vorzugsweise bei 3,0, erfolgt.

6. Verfahren nach Patentanspruch 1, 2, 3, 4 oder 5, dadurch gekennzeichnet, daß das Blei und das Silber aus dem Rückstand von Stufe (3) gewonnen werden.

7. Verfahren nach Patentanspruch 1, 2, 3, 4 oder 5, dadurch gekennzeichnet, daß das Blei aus der Stufe (3) gewonnen wird.

8. Verfahren nach einem der vorherigen Patentansprüche, dadurch gekennzeichnet, daß das Silber durch eine Auffällung (cementation) auf metallisches Zink, Eisen oder Blei zwischen der Stufe (b) und (c) gewonnen wird.

9. Verfahren nach einem der vorherigen Ansprüche, dadurch gekennzeichnet, daß ein Teil des Silbers aus dem das Bleisulfat enthaltenden Material durch Flotation vor der Stufe (a) gewonnen wird.

10. Verfahren nach einem der vorherigen Ansprüche, dadurch gekennzeichnet, daß in der Stufe (1) ein Molverhältnis von Sauerstoff zu Blei von größer als 0,5 besteht.

11. Verfahren nach einem der vorherigen Ansprüche, dadurch gekennzeichnet, daß die konzentrierte Chloridlösung aus einer gesättigten oder nahezu gesättigten Lösung bei Raumtemperatur eines oder mehrerer anorganischer Chloride in Wasser besteht.

12. Verfahren nach einem der vorherigen Ansprüche, dadurch gekennzeichnet, daß der Kalk in Stufe (1) im Überschuß vorliegt gegenüber dem Kalk in dem Niederschlag aus Stufe (c).

13. Verfahren nach Patentanspruch 12, dadurch gekennzeichnet, daß in der Stufe (1) frischer Kalk im Überschuß gegenüber dem Kalk im Niederschlag von Stufe (c) zugesetzt wird.

14. Verfahren zum Erschließen von Bleibeständen, wobei durch Zugabe von Kalk zu einer Chloridlösung mit Bleichlorid Bleioxichlorid ausgefällt wird und das Bleioxichlorid von der mageren Salzlösung abgetrennt wird, dadurch gekennzeichnet, daß in einer Stufe (1) der Niederschlag in einem Reaktor mit Sauerstoff und Kalk bei erhöhter Temperatur unter Bildung eines Kalzinats, das das meiste Blei als Calciumplumbat und/oder Bleioxid enthält, behandelt wird, daß in einer Stufe (2) durch Waschen des Kalzinats mit Wasser und/oder verdünnter Chloridlösung die löslichen Chloride herausgewashen werden und in einer Stufe (3) der erhaltene Rückstand mit dem Calciumplumbat und/oder Bleioxid aus der Salzlösung separiert wird.

15. Verfahren nach Patentanspruch 14, dadurch gekennzeichnet, daß die Chloridlösung irgendeine Salzlösung mit Bleichlorid ist.

16. Verfahren nach einem der vorherigen Patentansprüche, dadurch gekennzeichnet, daß der Rückstand aus der Stufe (3) mit frischem Wasser gewaschen wird, um restliche Chloride zu entfernen.

17. Verfahren nach einem der vorherigen Patentansprüche, dadurch gekennzeichnet, daß eine Komponente der Chloridlösung Calciumchlorid ist.

18. Verfahren nach Patentanspruch 17, dadurch gekennzeichnet, daß die Chloridlösung eine wässerige Lösung von Calciumchlorid und Natriumchlorid und/oder Magnesiumchlorid ist.

19. Verfahren nach einem der vorherigen Patentansprüche, dadurch gekennzeichnet, daß die Chloridlösung soviel Calciumchlorid enthält, daß das Molverhältnis von Calciumchlorid zu Bleisulfat größer als 4 ist.

20. Verfahren nach einem der vorherigen Patentansprüche, dadurch gekennzeichnet, daß in der Stufe (1) bei einer Temperatur oberhalb 325°C länger als 0,5 Stunden, vorzugsweise bei 400°C während 1 Stunde gearbeitet wird.

21. Verfahren nach einem der vorherigen Patentansprüche, dadurch gekennzeichnet, daß der Sauerstoff in Form von Luft angewendet wird.

22. Verfahren nach einem der vorherigen Patentansprüche, dadurch gekennzeichnet, daß die Chloridlösungen aus den Stufen im Prozeß wiederverwendet werden.
